

# UNITED STATES PATENT OFFICE.

JOHN J. GRAY, JR., OF ROCKDALE, TENNESSEE.

## BLAST-FURNACE PROCESS OF PRODUCING PHOSPHORUS AND PHOSPHORUS COMPOUNDS.

1,168,495.

Specification of Letters Patent. Patented Jan. 18, 1916.

No Drawing.

Application filed September 7, 1915. Serial No. 49,359.

*To all whom it may concern:*

Be it known that I, JOHN J. GRAY, Jr., a citizen of the United States, residing at Rockdale, in the county of Maury and State 5 of Tennessee, have invented certain new and useful Improvements in Blast Furnace Processes of Producing Phosphorus and Phosphorus Compounds; and I do hereby declare the following to be a full, clear, and exact 10 description of the invention, such as will enable others skilled in the art to which it appertains to make and use the same.

This invention relates to a continuous process of producing in a blast furnace, 15 phosphorus, together with compounds of phosphorus and various metals, and has for its object to provide a method which will attain these results when using natural phosphates in a manner more efficient, and less 20 costly than has been heretofore proposed.

With these and other objects in view the invention consists in the novel steps and combinations of steps more fully hereinafter disclosed and particularly pointed out in the 25 claims.

In order that the invention may be clearly understood it is said: In my prior Patent No. 831,427 dated Sept. 18, 1906, and entitled Manufacture of ferro-phosphorus I 30 have referred to various processes of producing ferro-phosphorus prior to said patent, and I have also disclosed a blast furnace method of producing ferro-phosphorus from natural phosphates. Among other

35 particulars this invention differs from the invention of my said patent and from the disclosure of the prior art in that its primary object is to produce phosphorus or phosphorus carrying vapors from natural phosphates in a blast furnace and its secondary object is to simultaneously produce in such a furnace phosphoreted compounds of phosphorus with the various metals, and metal alloys. It is well known that it has 40 been heretofore proposed to produce phosphorus itself in a blast furnace, but no one prior to my invention, so far as I am aware has ever succeeded in producing phosphorus from natural phosphates commercially in a 45 blast furnace and at the same time producing compounds of phosphorus with various metals or their alloys. It of course has, however, been proposed time and again to employ the more expensive electric furnace 50 in dealing with natural phosphates in the production of various compounds of phos-

phorus, but the limited capacity of electric furnaces as now known, and their relatively high cost of operation does not enable them to commercially compete with the less costly 60 blast furnace method to be disclosed below. Further, it has heretofore been thought so far as I am aware, where the silica was relied upon to expel the  $P_2O_5$  from the mineral phosphate, that wood charcoal was necessary. I have discovered that by properly proportioning the charge materials I can employ in a blast furnace successfully on a commercial scale, coke made from coal, and I have further discovered that if I add a 70 proper proportion of a metal or metal alloy, or of a metal ore to the charge, the process is greatly facilitated, in that the addition of such metal or metal ore maintains a molten bath which serves to keep up the temperatures of the exhausted refractory slag 75 materials, and to therefore maintain them sufficiently fluid to flow freely from the furnace when they are tapped off. This fluidity of the slag, further facilitates the escape of 80 the  $P_2O_5$  vapors as will appear below. In general any of the metals that are usually smelted in a blast furnace will be suitable 85 for this purpose, such for example as iron, copper, nickel, etc. However, when different metals, metal ores or alloys, are employed the proportions of the charge should be correspondingly varied as will be readily understood by those skilled in the art.

Briefly stated, the present invention consists in the continuous process of smelting in a blast furnace a mixture of tri-calcium phosphate or any natural phosphate, or phosphatic material, with sand or silicious material, to which has been added carbon 90 such as coke, charcoal, etc., or other suitable fuel, and to which has been also added lime or limestone, or other basic material, as well as a suitable metal such as iron, iron ores, copper, copper ores, nickel, nickel ores, or 95 alloys of said metals, making the necessary provision for air, and using only such quantities of each material as will be necessary to effect the physical and chemical changes 100 which end in the simultaneous production of chemical compounds of phosphorus and a metal, and of phosphorus vapors, which latter are conveyed away and treated under a separate operation to produce phosphorus 105 or phosphorus compounds.

In carrying out the invention of course an intimate and accurate analysis should be 110

made of all materials constituting the charge so as to accurately proportion the acids and bases. Only sufficient coke is used to provide sufficient heat to bring about the 5 desired chemical reactions between the various elements and to produce and maintain in the furnace more than enough carbon monoxide, CO, than is necessary for the de-oxidation of the phosphorus compounds liberated by the operation. The air is also used in quantities insufficient to completely ignite the coke or other carbon materials, and only in quantities sufficient to supply the oxygen necessary to the production of the requisite 10 heat in the furnace and to form a portion of the carbon monoxide. This deoxidizing agent gets part of its oxygen from the air and another part from the compounds liberated by the reactions which take place in the 15 furnace. Enough tri-calcium phosphate is used to yield sufficient phosphorus to be absorbed by the metals or alloys present, and to furnish in addition sufficient vapors of phosphorus to make the condensation of the 20 latter commercially profitable.

Silica in a suitable form is used as an acid to liberate the phosphoric acid,  $P_2O_5$  of the mineral phosphate from its alkaline base or bases, and in sufficient quantities to chemically satisfy said bases, or other compounds of the mixture, and in addition sufficient silica is employed to produce the desired fluidity in the slag. I may employ limestone or other cheap sources of basic material, in such amounts as are necessary to neutralize the acid materials present when they are in excess, I also endeavor to make the quantity small, as it is best to make the silicic acid take up as much of the bases from the phosphates as it is possible to do, and thus liberate the highest possible percentage of phosphorus.

With a charge of the character above, and heated to the high temperatures of a blast furnace the silicic acid attacks the phosphates, combines with their basic materials, liberates the phosphoric acid  $P_2O_5$ , and forms compounds making up the slag. The  $P_2O_5$  thus liberated in a reducing atmosphere of  $CO$ , is deoxidized to phosphorus vapors. The metal or alloys being in insufficient quantities to take up more than say 40% or 50% of the phosphorus liberated, and the remainder of the said phosphorus having nothing with which it can combine, it passes out with the other furnace gases and may be subsequently recovered as red phosphorus, as ortho phosphoric acid, or in any other desired form. In the meantime the metals present form a molten pool, which serves to impart heat to the slag, and therefore to maintain the latter more fluid than would be the case if no metals were present. Said metals accordingly hot only render the slag more easy to tap from the

furnace but it is found in practice that their presence causes a greater liberation of  $P_2O_5$  from the molten mass, than would otherwise take place. In other words, the  $P_2O_5$  is probably mechanically held in the slag and molten mass, owing to its high surface tension, and the more fluid is the slag, the more readily does such vapors escape therefrom. 70

The phosphoreted metals may be tapped out at the bottom of the furnace and run off as is pig iron, or ferro-phosphorus, and the slag is also run off at regular intervals, in a manner well known. 75

A more definite understanding of my process will be had from the following: About eight pounds of air will ignite say two thirds of a pound of coke, to form  $\text{CO}_2$ , and will also oxidize say one third of a pound of coke to form  $\text{CO}$ . I have found that by using preheated air at the rate of say eight pounds to one pound of coke, and thus producing  $\text{CO}_2$ , and  $\text{CO}$  gases as above mentioned, and using coke to the amount of say 40% of the total charge, I will get sufficient heat for the desired reactions and in addition I will obtain sufficient  $\text{CO}$  gas to maintain at all times the necessary reducing atmosphere. By thus maintaining the proper temperature and reducing atmosphere in the furnace the desired reactions take place, and by continuously charging the proper proportioned materials into the top of the furnace and by discharging at the bottom of the furnace at regular intervals the end products which accumulate in this zone, the process is rendered continuous. The heated or molten metal which is being continuously heated and melted above the fusion zone, drips through or comes into contact with the rising phosphorus vapors, and absorbs said vapors to form various metal phosphids.

If the ordinary natural phosphates and iron ore are employed a specific charge may be prepared as follows: Using for example a phosphate rock consisting of say 75% tricalcium phosphate having 40% CaO combined with  $P_2O_5$  to form the  $Ca_3.P_2O_8$ , and supposing 16% of said rock consists of carbonates, sulfates and fluorids of calcium, while say 4½% of said rock consists of silica,  $SiO_2$ , and say 4½% consists of  $Fe_2O_3$  the proportions of the charge would be as follows: air, 1472 pounds; coke, 184 pounds; natural phosphates, 140 pounds; sand or flint (containing 90%  $SiO_2$ ), 64 pounds; iron ore (containing 50% Fe and 18%  $SiO_2$ ), 60 pounds;  $CaCO_3$  (if found necessary on account of incomplete reactions), 12 pounds.

Supposing the reactions are all complete the 184 pounds of coke considered as pure carbon would in its major part ignite to form  $\text{CO}_2$  gas with the oxygen of the air, 130

and thereby produce the desired temperature in the furnace. This said coke would also in its minor part combine with the remaining oxygen of the air, as well as with some of the oxygen of the evolved compounds to form sufficient CO gas to reduce all the deoxidizable compounds of the charge, while the gases discharged from the furnace will contain sufficient heat to pre-  
heat the air employed for a succeeding charge if they are passed through the usual stoves.

The various constituents of the charge may be stated to react about as follows: 105  
15 pounds of tri-calcium phosphate, together with the 22.4 pounds of calcium fluorid, calcium carbonate and calcium sulfate that are physically combined with the tri-calcium phosphate are decomposed by the silicic acid present. Of this acid 6.3 pounds are carried by the phosphate rock, 10.8 pounds are carried in the iron ore, and 57.6 are carried by the sand. In all 75 pounds of the  $\text{SiO}_2$  combine with the total 70 pounds of CaO present to form 145 pounds of  $\text{CaSiO}_3$ , and thus cause the liberation of 48.9 pounds of  $\text{P}_2\text{O}_5$ , as well as 8.4 pounds of fluorin, carbonic acid gas and sulfur dioxid. This  $\text{P}_2\text{O}_5$ , is, of course, at once deoxidized in the reducing atmosphere to form 21 pounds of phosphorus, the CO present thus taking up 27.09 pounds of oxygen from the  $\text{P}_2\text{O}_5$ . The 30 pounds of iron present coming into contact with the 21 pounds of phosphorus vapor absorbs 8.4 pounds of phosphorus to form 38.4 pounds of iron phosphids such as  $\text{FeP}$ ,  $\text{Fe}_2\text{P}$ , and  $\text{Fe}_3\text{P}$  which together will contain say 22% of phosphorus. The 30 pounds of iron having absorbed 8.4 pounds of phosphorus the remaining 12.6 pounds of phosphorus goes over as vapors with the other gases, and may be recovered as red phosphorus or in any desired form. Accordingly, after having started the furnace with 1472 pounds of air, 184 pounds of coke, 140 pounds of phosphate rock, 64 pounds of sand or flint and 60 pounds of iron ore, or a total of 1920 pounds, the reactions being complete, I end with 1691 pounds of gases (some or all of which may be used to pre-heat the succeeding charge of air), as well as with 12.6 pounds of phosphorus vapors, 38.4 of iron phosphids and 178 pounds of  $\text{CaSiO}_3$ . In practice these reactions are to a slight degree varied by differing temperatures and by differing physical and mechanical conditions. The reactions between the tri-calcium phosphate and the silica are really never complete, for a small amount of the phosphoric acid always becomes entangled in the slag mass which probably takes on more lime than would otherwise be the case, instead of releasing that present, and probably for this and other reasons the slag sometimes becomes too acid and

gives trouble around the twyers. Here the use of a small amount of carbonate of lime becomes of great importance, for by using the above mentioned 12 pounds of  $\text{CaCO}_3$ , the acid condition of the slag is obviated. 70 In other words, whenever in the judgment of the expert furnace man the equilibrium between the acids and bases has become disturbed a small portion of calcium carbonate is employed, but inasmuch as the use 75 of the carbonate of lime cannot be made immediately effective it being charged in at the top of the furnace, its use must be anticipated, whenever possible, and the expected relief awaited.

In stating in detail the above reactions, of course, I have not explained a few insignificant complications involving complex chemical compounds, but they do not materially change or interfere with the process.

It will thus be seen that by following the foregoing process I avoid the great objection which others have encountered in attempting to produce phosphorus from natural phosphates in a blast furnace and which is caused by the materials being too refractory to be handled in the old way. I avoid this objection largely by the use of the metals or ores or the alloys above mentioned 90 which seems to render the slag as well as the molten mass more fluid at the point of discharge than would otherwise be the case at the temperatures of a blast furnace and also which seem to increase the output of 100  $\text{P}_2\text{O}_5$ . At the same time it will further be observed that I produce two valuable products namely phosphorus and the chemical compounds of phosphorus with the various metals and their alloys. Especially is this 105 process important in connection with the phosphoreting of metallic copper its alloys and copper ores but of course in that case the proportions of the charge given above would have to be varied as it would be when 110 other metals or their alloys are employed. In all cases it is very desirable that an experienced furnace man carry out the process, and that an intimate accurate chemical knowledge of all the materials be had.

It is evident that by increasing the quantity of phosphate rock and silica and coke, or by decreasing the amount of iron and coke used in the process, I can produce a surplus of phosphorus vapor or by making 115 other obvious changes I can lessen the quantity of phosphorus vapor produced at will.

Since when employing various metals and ores the problem is one largely a matter of readjusting the equilibrium between the acid and bases, it is obvious that those skilled in the art may vary the details of the process, as well as the steps disclosed without departing from the spirit of the invention, and therefore I do not wish to be lim- 120

ited to the above disclosure, except as may be required by the claims. In fact it is clear that instead of a major portion of the phosphorus vapors being allowed to leave the furnace, and a lesser portion being taken up by the metals these proportions may be reversed and a major portion of the phosphorus vapors may be taken up by the metals and a lesser portion allowed to leave the furnace. Especially would this be the case when metallic copper, copper ores or copper alloys are employed.

What I claim is:

1. The process of simultaneously producing in a blast furnace phosphorus and metal phosphids from a natural phosphate, which consists in charging said furnace with a suitable mixture containing said phosphate, sufficient silica to liberate the desired amount of phosphorus, metal sufficient to make the desired amount of phosphids and to produce the desired fluidity in the slag but insufficient to take up all the liberated phosphorus, and sufficient carbon to produce the desired reacting temperature as well as a reducing atmosphere in the furnace; and feeding to said charge only sufficient air to produce said temperature and reducing atmosphere, substantially as described.
2. The process of simultaneously producing phosphorus and metal phosphids from a natural phosphate in a blast furnace, which consists in charging said furnace with a suitable mixture containing said phosphate, sufficient silica to liberate the desired amount of phosphorus, metal sufficient to make the desired amount of phosphids and to produce the desired fluidity in the slag but insufficient to take up more than eighty per cent. of the liberated phosphorus, and sufficient carbon to produce the desired reacting temperature as well as a reducing atmosphere in the furnace; and feeding to said charge only sufficient air to produce said temperature and reducing atmosphere, substantially as described.
3. The process of simultaneously producing phosphorus and phosphids which consists in charging a blast furnace with a mixture containing a natural phosphate, sufficient silica to liberate a predetermined quantity of phosphorus, metal in the form of an ore sufficient to take up a predetermined per cent. of the liberated phosphorus and to produce the desired fluidity in the slag, but insufficient to take up a predetermined

other quantity of said phosphorus, and sufficient carbon to bring about the desired reactions while supplying a reducing atmosphere in the furnace, and so controlling the air fed to the furnace as to maintain said reducing atmosphere therein, substantially as described.

4. The process of simultaneously producing phosphorus and phosphids which consists in charging a blast furnace with a mixture containing a natural phosphate, sufficient silica to liberate a predetermined quantity of phosphorus, metal in the form of an ore sufficient to take up more than ten per cent. of the liberated phosphorus and to produce the desired fluidity in the slag but insufficient to take up a substantial major quantity of said phosphorus, and sufficient carbon to bring about the desired reactions and to supply a reducing atmosphere in the furnace; and so controlling the air fed to the furnace as to maintain said reducing atmosphere therein, and adding to said charge when found necessary a small quantity of a basic material to render the slag more fluid.

5. The process of simultaneously producing phosphorus and phosphids which consists in charging a blast furnace with a mixture containing a natural phosphate, sufficient silica to liberate a predetermined quantity of phosphorus, iron sufficient to take up more than ten per cent. of the liberated phosphorus, but insufficient to take up a predetermined major quantity of said liberated phosphorus, and sufficient carbon to bring about the desired reactions while supplying a reducing atmosphere in the furnace; and so controlling the air fed to the furnace as to maintain said reducing atmosphere therein, substantially as described.

6. The process of simultaneously producing phosphorus and phosphids which consists in charging a blast furnace with predetermined quantities of a phosphate, silica, carbon, and a metal in a suitable form; and causing the contained phosphorus to be liberated and a predetermined portion thereof to enter said metal and a predetermined portion to leave the furnace in the form of a vapor, substantially as described.

In testimony whereof I affix my signature, in presence of two witnesses.

JOHN J. GRAY, JR.

Witnesses:

HYLEMAN A. WEBSTER,  
D. R. GRAY.